

Feb. 16, 1971

K. LINDERS

3,563,081

FORGING OF RAILROAD VEHICLE AXLES

Filed Aug. 21, 1968

2 Sheets-Sheet 1

Fig. 1



Fig. 2



Fig. 3



Fig. 4



Fig. 5



Fig. 6



INVENTOR.  
KARL LINDERS

BY Glascott, Downing & Sebold  
ATTORNEYS.

Feb. 16, 1971

K. LINDERS

3,563,081

FORGING OF RAILROAD VEHICLE AXLES

Filed Aug. 21, 1968

2 Sheets-Sheet 2



INVENTOR.  
KARL LINDERS

BY Glascock, Downing & Sebco  
ATTORNEYS.

## 1

3,563,081

**FORGING OF RAILROAD VEHICLE AXLES**  
Karl Linders, Buttgen, near Neuss, Germany, assignor to  
Schloemann Aktiengesellschaft, Dusseldorf, Germany,  
a German company

Filed Aug. 21, 1968, Ser. No. 754,242  
Claims priority, application Germany, Sept. 5, 1967,  
Sch 41,260  
Int. Cl. B21k 1/10

U.S. Cl. 72—374

3 Claims

### ABSTRACT OF THE DISCLOSURE

A method of forging billets for railway-coach axles, the diameter of the axle between the wheel seats being either the same as the diameter of the journals or different, wherein the billets are first forged to round material of a diameter equal to the finish-forged diameter of the wheel seats, and the round material is then finish-forged in a drop-forging press in at least two working strokes, a portion of the round material of a length at least equal to the distance between the wheel set upon the round material being finish-forged in one stroke.

This invention relates to a method of forging billets into railway-coach axles, which, after the forging, will be either of the same diameter between the wheel seats and on the journals, or will be, on the journals, of a diameter different from the diameter between the wheel seats.

Railway-coach axles are usually forged from a billet under a forging hammer, and at times in one operation. This operation is divided into the forging of the journals, of the wheel seats, and of the intermediate piece connecting the wheel seats with one another. Each part of the operation imposes special requirements on the forging tools, so that these cannot by any means always ensure optimum operative conditions in all parts of the operation at the same time, and the forging operation is more or less dependent upon the skill of the workmen operating the forging hammer, that is to say, the individual railway-coach axles, after being forged, usually exhibit very great deviations from one another in their dimensions. This is very objectional for their subsequent treatment in automatic lathes.

The object of the present invention is therefore to provide a process for the forging of railway-coach axles with exactly the same dimensions and properties, and under optimum conditions.

This aim is substantially attained according to the invention by the feature that the billets are first forged to round material, the diameter of which is equal to the diameter of the wheel seats of the finish-forged railway-coach axles, and the round material is then further finish-forged in a drop-forging press, in at least two working strokes, wherein, from the intermediate piece of the railway-coach axle connecting the wheel seats with one another, a piece of a length which at most is equal to the distance between the wheel seats upon the round material before the finish-forging thereof, is finish-forged in one stroke. The forging of the railway-coach axles is now divided into the forging of the round material, the finish-forging of the wheel seats, and the forging of the intermediate piece connecting the wheel seats with one another, and the forging of the journals. The diameter of the round material is therefore the final dimension of the finish-forged wheel seats, so that two pieces of the round material of corresponding length and/or breadth are no longer further forged as later wheel seats and brought by forging out or stretching the round material located between these positions to a desired distance from one an-

## 2

other, that is, to the gauge or track width of the railway-coach. Advantageously the forging of round material, and the forging out or stretching of a part of the round material in the die or swages are simple forging operations at times, so that the process according to the invention ensures undisturbed operation.

In a further development of the invention it is provided that the railway car axles should be straightened in the drop-forging press after being forged.

10 Further features of the invention are presented in the following description of one example of the process according to the invention, and in a following drawing of the apparatus necessary for carrying out the process.

15 FIG. 1 shows the swage or drop-forging die in a general view;

FIGS. 2 to 6 are diagrammatic representations of the steps of the process; and

FIG. 7 is a plan view of the forging plant as a whole.

From a rotary furnace A, square billets B, after they 20 have been heated to forging temperature, are drawn out individually by a billet-drawing machine C, transported into the range of action of a gripping arm D, and there dropped. The gripping arm D brings the square billets B into the middle of a free-form forging press E, so that the 25 square billets B can be seized by a manipulator F, and forged, in the free-form forging press E, into round material b, of a diameter equal to the diameter of the wheel seats of the finish-forged railway-coach axles.

From the free-form forging press E the round material 30 b is supplied, at a temperature between 1100° and 1150° C., by means of a roller table, to a further gripping arm d, which brings this round material b into the middle of a drop-forging press G, in such a way that it can be seized by a manipulator H pertaining to the drop-forging 35 press G.

The round material is then moved by the manipulator H so far into a sleeve or die 1 of the drop-forging press G that less than half the length of the round material projects out of the sleeve 1 at the next stroke of the drop-forging press G. The sleeve 1 is of a hollow cylindrical form, and has been bored to the diameter of the wheel seats on the side remote from the manipulator H, and serves merely for the forging of the round material between the wheel seats, so that the round forging material 40 b is stretched, in the next forging operation, with a plurality of working strokes of the drop-forging press G, in the sleeve 1, without the part of the round material b, which is afterwards to become the wheel seat being deformed. Before the next forging operation the round material b is drawn so far out of the sleeve 1 by the manipulator H that after this forging operation, as illustrated in FIG. 2, with a plurality of working strokes, of the intermediate piece between the wheel seats, more than half, and at the same time a piece up to one wheel seat, has 45 been forged out or finish-forged.

Then, as illustrated in FIG. 3, the round material b is moved by the manipulator H into a further sleeve 2 of the drop-forging press G, which in shape is a mirror image of the sleeve 1, and serves solely for the forging of the journals. It is in fact moved so far that after the succeeding forging operation, with a plurality of working strokes, the journal, on the wheel seat, except for which the intermediate piece has already been forged is finish-forged.

For the forging of the second half of the round material b, the forging is turned round, and with the part that is still round material, is placed in the sleeve 1 so far that in the next forging operation of the drop-forging press G, a further part of the intermediate piece between the wheel seats is finish-forged, enlarging the hitherto forged-out part, without transition, or in other words 50 seamlessly.

Before the next forging operation, the remainder of the intermediate piece, as illustrated in FIG. 4, is finish-forged, or, in other words, the wheel seats, after the stretching of the intermediate piece occurring during the forging, have been given the desired distance from one another, namely the track width of the railway coach.

After the forging out of the intermediate piece, the forging is moved by the manipulator H out of the sleeve 1, and so far into the sleeve 2, that, as illustrated in FIG. 5, during the next forging operation of the drop-forging press G, the second journal, not yet forged out, is finished-forged, and thus at the same time the remainder of the railway-coach axle is finish forged, so that the latter, after being straightened in a straightening sleeve 3 of the drop-forging press G, as illustrated in FIG. 6, can be supplied by means of tongs to a cooling bed J.

The displacement path of the manipulator H, or, in other words, the path by which the forging is moved from time to time in a sleeve, is yielded from the equality of volumes of the forging before and after deformation.

The intermediate piece and the journals of a railway-coach axle are preferably, according to the present process, forged exactly centrally to the wheel seats, since the wheel seats are machined in each sleeve, and the railway-coach axles, when being forged with the wheel seats, or with a portion of the billets forged out to the diameter of the wheel seats, bear in the sleeves 1 and 2.

I claim:

1. A method of forging billets into railway vehicle axles, comprising the steps of: heating the billets to forging temperature, forging the billet, in a free-form forging press, into round material, corresponding in diameter over its entire length, to the ultimate diameter of the finished wheel seats, thereupon forging, in the same heat, in a drop-forging press, one-half of the axle, in two operations, the first operation being the finish-forging in a die of at least half the round material between the wheel

seats, and the second operation being the finish-forging of the journal of the same half-axle in another die, the half-finished axle then being turned, and the other half-axle being finish-forged by a repetition of the same two operations.

2. Means for forging billets into railway vehicle axles, comprising: a free-form forging press with straight saddles for the round-forging of the billet, a drop-forging press with two open dies, the length of each die being less than half the length of the axle, the diameter of the forging groove of one of the said dies being in one part about equal to the diameter of the wheel seats and in the other part to the diameter of the axle between the wheel seats, and the forging groove of the other die being constructed as a mirror image of the first die.

3. Means for forging billets into railway vehicle axles as claimed in claim 2, the two said open dies being located one to the right and the other to the left of the forging axis of the drop forging press, and the forging means further comprising a straightening die arranged between the two said open dies, the said straightening die consisting of an upper straightening stamp located in the axis of the press, and two lower straightening anvils located one to the right and the other to the left of the axis of the press.

#### References Cited

##### UNITED STATES PATENTS

2,512,484 6/1950 Cornell ----- 72—374

##### FOREIGN PATENTS

772,724 4/1957 Great Britain ----- 72—377

LOWELL A. LARSON, Primary Examiner

U.S. CL. X.R.

72—377